

March 24, 1953

I. F. SALMINEN ET AL

2,632,701

ULTRAVIOLET FILTER ON PHOTOGRAPHIC LAYERS

Filed May 4, 1949



*Ilmari F. Salminen  
Charles F. H. Allen*

INVENTORS

BY *Daniel J. Mayne*  
*R. Frank Smith*  
ATTORNEYS

## UNITED STATES PATENT OFFICE

2,632,701

## ULTRAVIOLET FILTER ON PHOTOGRAPHIC LAYERS

Ilmari F. Salminen and Charles F. H. Allen,  
Rochester, N. Y., assignors to Eastman Kodak  
Company, Rochester, N. Y., a corporation of  
New Jersey

Application May 4, 1949, Serial No. 91,422

4 Claims. (Cl. 95—2)

1

This invention relates to a method of protecting multi-layer photographic elements against the action of ultra-violet light and to multi-layer elements containing ultra-violet filtering materials.

It is known that color photographs on multi-layer photographic material, particularly where the dye images are formed in sensitive emulsion layers by color development, are susceptible to fading and discoloration by the action of ultra-violet light to which the photographs are subjected during viewing. It is also known that the residual couplers contained in the emulsion layers after formation of the picture images in certain processes, are attacked by ultra-violet light and form a stain which is undesirable in the finished photograph. The action of ultra-violet light on finished color photographs is particularly noticeable in positive prints on paper or other opaque supports since this type of print is frequently viewed in daylight where there is a high content of ultra-violet radiation.

It is also known that color photographs, especially where the dye images are formed by color development, can be protected from the fading and discoloration caused by ultra-violet light by applying to the finished color photograph a layer of gelatin or other colloidal material having therein an ultra-violet absorbing material. A process of this type in which aesculin, quinine, primuline, disalicylbenzidine, etc., are used as ultra-violet absorbing materials in a gelatin overcoating layer is described in British Patent 565,929. Processes of this type have the objection that the ultra-violet filtering material must be applied from colloidal solution, e. g., gelatin, and an application of this character requires coating machinery and necessitates an expensive and additional coating operation after the processing of the color print is finished.

It is therefore an object of the present invention to provide a simple method for protecting finished multi-layer photographic color prints against the action of ultra-violet light. A further object is to provide finished multi-layer color photographs in which the color image is not appreciably subject to fading or discoloration by the action of ultra-violet radiation. Other objects will appear from the following description of our invention.

These objects are accomplished by applying to the outermost layer of a multi-layer photo-

graphic element, where the outermost layer is gelatin, an aqueous non-colloidal solution of a water-soluble sulfonated organic compound which is adsorbed to gelatin and which is absorbent of ultra-violet light of wave length between 300 and 400 millimicrons but transmissive of light of wave length longer than 400 millimicrons. In particular, we have found that water-soluble sulfonic acid salts of compounds of the following structure are especially useful for application to the finished gelatin layer from non-colloidal solution:



15 where

X=—CH=CH—, or represents a single chemical bond

R=a mononuclear aryl radical

Y=benzoyl or s-triazinyl

By "mononuclear aryl radical" we mean a radical such as phenyl, hydroxyphenyl, hydroxytolyl and sulfonated derivatives of these radicals.

By "benzoyl" we mean the radial,  $C_6H_5CO-$  or substituted benzoyl radicals such as hydroxyl benzoyl, hydroxy tolulyl or sulfonated derivatives of these radicals.

The accompanying drawing is a sectional view of a finished photographic element comprising three finished emulsion layers overcoated with a gelatin layer containing an ultra-violet absorber applied according to our invention.

The following compounds are illustrative of those suitable for use according to our invention.



Di-(2'-hydroxy-4'-methylbenzoyl)-benzidine sodium sulfonate



Di-(2'-hydroxy-3'-methylbenzoyl)benzidine sodium sulfonate



Bis-(4-hydroxy-3-carboxyphenyl sulfonyl)-benzidine



4,5-diphenyl-2-imidazolondisulfonic acid (Na salt)



4,4'-di-(phenylcarbamido)-stilbene-2,2'-disulfonic acid (Na salt)



4,4'-di-(3'', 5''-dihydroxy-s-triazinylamino)-stilbene-2,2'-disulfonic acid (Na salt)



These ultra-violet absorbing materials have a high ultra-violet absorption in the regions between 300 and 400 millimicrons but relatively little absorption in the visible region at wave length longer than 400 millimicrons. We prefer to apply them to a multi-layer photographic element such as those described in Mannes and Godowsky U. S. Patent 2,304,940, or Jelley and Vittum 2,322,027, by coating from a simple aqueous solution after the multi-layer element has been developed and fixed. The solution of the ultra-violet absorber may be used as the final stage of the processing of the material described in the U. S. Patents 2,304,940 or 2,322,027, that is, after the final wash but before drying. However, if the multi-layer element has been washed and dried, the ultra-violet absorber may be applied after drying and the photograph again rinsed and dried.

The following example illustrates a method of applying our ultra-violet absorbing material.

After the final washing step of the process described in U. S. Patents 2,304,940 or 2,322,027, the photographic element is treated in the following solution for 10 minutes followed by a 1-minute rinse and finally a squeegeeing operation.

Grams  
Disalicylbenzidine sodium sulfonate ----- 10  
Water to 1 liter.

The pH of the ultra-violet absorber solution is preferably adjusted to 7.0 or 8.0 by the addition of either sodium hydroxide or hydrochloric acid as required. After treatment for about 10 minutes as indicated, the element is dried in the normal manner.

With some of the ultra-violet absorbers, it is desirable to follow the bathing operation by a brief treatment, e. g., two minutes, in an aqueous buffer solution at a pH of 3.0 to 5.0. In some cases this prevents excessive yellowing of the

65

70

75

Our invention will now be described by reference to the accompanying drawing. As shown therein a support **10** is coated with superposed layers **11**, **12** and **13** containing respectively cyan, magenta and yellow dye images. These are finished photographic layers, that is, developed and fixed emulsions after exposure and color development, and removal of residual silver and silver halide. The outermost layer **13** has on it a layer **14** of gelatin containing the sulfonic acid salt of disalicylbenzidine, the sulfonic acid salt

residual magenta coupler in the multi-layer element on moist storage of the finished print. The acid buffer treatment has nothing to do with the adsorption of the ultra-violet absorber.

It has been found advantageous to incorporate in the uppermost gelatin layer of the multi-layer element to which the ultra-violet absorber is applied, a mordant for the ultra-violet absorber. Polyvinyl pyridine methyl p-toluenesulfonate has proven particularly suitable as a mordant for the various sulfonated ultra-violet absorbers which we propose to use. Such a mordant binds the ultra-violet absorber more tightly to the gelatin layer and permits a washing operation after the application of the absorber. By use of this expedient the absorber may be introduced at some stage of the process before the final wash and this obviates the necessity for the acid-buffer treatment described above.

The preparation of disalicylbenzidine sodium sulfonate is illustrated by the following example and other compounds which we propose to use as ultra-violet absorbers may be similarly prepared.

A solution of 40 g. of benzidine, 100 g. of phenyl salicylate and 500 g. of  $\alpha$ -chloronaphthalene was heated in a 1-l. flask attached to a 12-inch Vigreux column so that the phenol distilled (180-200°). When no more phenol distilled, the reaction mixture was heated strongly until the temperature of the distilling vapours was between 235-240° C., at which point the reaction was considered to be complete. On cooling to room temperature, the product separated. It was collected by filtration and washed with dioxane and then acetone. The yield of light gray product was 88.5 g. (98); M. P. 320-324°.

Eighty grams of finely pulverized disalicylbenzidine were added to 480 ml. of concentrated sulfuric acid, and the reaction mixture was maintained at an inside temperature of 88-93° C. for 3.5 hours. It appears as a clear dark brown solution at this point. It was poured with good stirring into 2400 ml. of 10% potassium chloride, using Dry Ice as an internal coolant. After standing for one hour to allow for coagulation, the product was collected by filtration. The filter cake was boiled with 1-l. of methanol and again filtered. The crude sulfonic acid thus obtained was taken up in 600 ml. of 10% sodium carbonate solution and decolorized twice, using 15-20 g. portions of Norite, after which 60 g. of sodium chloride was added to the boiling solution with good stirring. The stirring was continued while cooling to room temperature and the mixture was then allowed to stand overnight. The crystalline white product was collected by filtration and washed with methanol. The yield was 30 g. The filtrate was heated to boiling and 100 g. of sodium chloride was added with vigorous stirring and treated as before: after filtering and drying 66 g. of product was obtained. The combined yield was 96 g. (80% of the theory of 119 g.).

Our invention will now be described by reference to the accompanying drawing. As shown therein a support **10** is coated with superposed layers **11**, **12** and **13** containing respectively cyan, magenta and yellow dye images. These are finished photographic layers, that is, developed and fixed emulsions after exposure and color development, and removal of residual silver and silver halide. The outermost layer **13** has on it a layer **14** of gelatin containing the sulfonic acid salt of disalicylbenzidine, the sulfonic acid salt

having been applied from an aqueous non-colloidal solution.

It will be understood that the examples and modifications included herein are illustrative only and that our invention is to be taken as limited only by the scope of the appended claims.

We claim:

1. The method of applying an ultra-violet protective agent to a developed and fixed multi-layer photographic element having superposed dye images and having a gelatin layer as the outermost layer which comprises applying to said gelatin layer from aqueous non-colloidal solution, a water-soluble sulfonic acid salt of a compound having the following structure:



in which X is selected from the class consisting of  $-CH=CH-$  and a single chemical bond, R represents a mononuclear aryl radical and Y is selected from the class consisting of benzoyl and s-triazinyl radicals, said compound being adsorbed to the gelatin and being absorbent of ultra-violet light of wave length between 300 and 400 millimicrons but transmissive of light of wave length longer than 400 millimicrons.

2. The method of applying an ultra-violet protective agent to a developed and fixed multi-layer photographic element having superposed dye images and having a gelatin layer as the outermost layer which comprises applying to said gelatin layer from aqueous non-colloidal solution, a water-soluble sulfonated disalicylbenzidine which is adsorbed to the gelatin and which is absorbent of ultra-violet light of wave length between 300 and 400 millimicrons but transmissive of light of wave length longer than 400 millimicrons.

3. The method of applying an ultra-violet protective agent to a developed and fixed multi-

layer photographic element having superposed dye images and having a gelatin layer as the outermost layer which comprises applying to said gelatin layer from aqueous non-colloidal solution, disalicylbenzidine sodium sulfonate which is adsorbed to the gelatin and which absorbs ultra-violet light but transmits visible light.

4. A finished photographic element comprising a paper support having thereon three superposed developed and fixed gelatin emulsion layers each containing coupled dye images, said dye images being subject to fading by the action of ultra-violet light, an outermost layer of said element being a gelatin layer containing a polyvinyl pyridine mordant and also containing a water-soluble sulfonic acid salt of a disalicylbenzidine which is adsorbed and mordanted to said gelatin and is absorptive of substantially all ultra-violet light of wave length between 300 and 400 millimicrons but transmissive of light of longer wave length than 400 millimicrons.

ILMARI F. SALMINEN.  
CHARLES F. H. ALLEN.

#### REFERENCES CITED

The following references are of record in the file of this patent:

#### UNITED STATES PATENTS

| Number    | Name    | Date         |
|-----------|---------|--------------|
| 1,568,511 | Lehmann | Jan. 5, 1926 |

#### FOREIGN PATENTS

| Number  | Country       | Date          |
|---------|---------------|---------------|
| 333,933 | Great Britain | Aug. 25, 1930 |
| 493,308 | Great Britain | Oct. 6, 1938  |
| 524,377 | Great Britain | Aug. 5, 1940  |
| 565,929 | Great Britain | Dec. 6, 1944  |